

## UNITED STATES PATENT OFFICE

2,510,650

COMPOSITION FOR RECTIFYING HALIDE  
SALT BATHSIsaac Laird Newell, Wethersfield, Conn., assignor  
to Heatbath Corporation, Indian Orchard,  
Mass., a corporation of MassachusettsNo Drawing. Application October 3, 1947,  
Serial No. 777,848

11 Claims. (Cl. 252—71)

1

This invention relates to a method of maintaining the efficiency of salt baths which are composed substantially of halides and are commonly used in the treatment of certain metals. By halides in the present disclosure are meant the elements fluorine, chlorine, bromine, and iodine of group 7 of the periodic table.

Such salt baths as are composed of mixtures of alkali metal and alkaline earth halides are commonly fused and used as media for the heat treatment of steels and other metals. It is well known in the case of steel that after a certain period of use a bath becomes decarburizing to the metal. One object of this invention is to provide a simple, inexpensive and effective method for maintaining the efficiency of the salt baths to eliminate decarburization and to do this without the disadvantages attending prior art procedures so far as they are known to me.

Said salt baths are also used in the treatment of copper alloys and nickel alloys and when used for a certain period with these metals become alkaline to a degree that will cause pitting, etching and staining of the metal being treated.

In maintaining the efficiency of halide baths it is common in the language of the trade to speak of keeping a bath neutral to the metal. In other words a neutral bath will neither carburize nor decarburize steel, nor will it cause pitting and etching of other metals which are commonly treated in said baths. The term neutral as used in this disclosure is intended to have this meaning. Further, the process of maintaining this type of bath neutral is called a process of rectification.

When such baths are no longer neutral, it is customary to discard the baths or to treat the baths with materials such as silica or silicon carbide which will cause the formation of insoluble materials which are then removed as a sludge from the molten salt, but with attendant loss of salt along with the sludge. This method also limits production as the de-sludging usually requires lowering the temperature below the working temperature. The baths also increase in viscosity due to the materials added.

Another method of treatment heretofore used consists in immersing a carbon rod in the molten bath. This method does not give complete rectification under all conditions and presents some hazards since small pieces of carbon breaking from this rod may come in contact with the metal being treated and cause hard spots, or even fused metal in the high temperature baths.

My invention makes use of materials which completely neutralize salt baths and yet are not open to the objections noted above.

I have found that a molten salt bath such as is composed substantially of alkali halides, alkaline earth halides, or a mixture of alkali and

2

alkaline-earth halides which has become alkaline and thus decarburizing to steel can be rectified and made neutral and nondecarburizing to steel by treating the molten salt baths with a compound, nongaseous at standard temperatures and pressures, substantially inert with respect to the metals being treated, but reactive with their oxides, containing fluorine as a component element and at least one other element capable of forming an oxide neutral or acidic in reaction. By standard temperature and pressure is meant 0° centigrade temperature and 760 millimeters pressure.

Among nongaseous compounds containing fluorine found to be suitable as rectifiers of molten salt baths are those containing boron as one of the elements such as ammonium fluoroborate; sodium fluoroborate; potassium fluoroborate; lithium fluoroborate; calcium fluoroborate; magnesium fluoroborate; strontium fluoroborate and barium fluoroborate. Other nongaseous fluorine compounds suitable as rectifiers may have silicon as one of the elements such as ammonium fluosilicate; sodium fluosilicate and potassium fluosilicate. Suitable compounds containing fluorine may also contain carbon such as polytetrafluoroethane. These materials are not intended to be a complete list of the compounds included within the scope of this invention, but are given merely to show the wide variety of compounds that act satisfactorily as rectifiers.

It is believed that the mechanism of rectification takes place in the following manner:

(1) The compound containing fluorine reacts selectively with the oxides present to reduce them to the elemental state.

(2) The newly formed metals react with the fluorine to form new stable neutral compounds which will be either volatile at this bath temperature or soluble in the molten bath.

(3) The new oxides formed are either neutral or acidic in reaction, and when acidic, they further react with any alkali present to form a new neutral compound.

Herewith are several examples within the scope of this invention.

*Example I*

A salt bath used for the hardening of a steel, the composition of which is carbon 0.45%, manganese 0.75%, phosphorus 0.035%, and sulfur 0.040%, is composed of 45% potassium chloride and 55% sodium chloride and is rectified by the use of potassium fluoroborate. The salt bath is fused by heating to the hardening temperature of the steel, 1525° F., and when chemical analysis shows the bath to have an excessive alkalinity, which is above approximately 0.5% when calculated as sodium oxide, the bath is rectified by adding potassium fluoroborate. This is added in small quantities with stirring. Sufficient potas-

slum fluoborate is added to reduce the alkalinity to below the required limit. When an article of steel having the above composition is heated for an hour at 1525° F. in the salt bath, rectified as described, and quenched in oil, then the surface will show no pitting or decarburization to have taken place in the salt bath.

*Example II*

A salt bath composed of 77% barium chloride and 23% sodium chloride is used to harden a steel composed of carbon 0.40%, manganese 0.75%, nickel 1.25% and chromium 0.60%, by heating it at a temperature of 1500° F. in the bath and quenching the steel in oil. The salt bath is kept in a neutral condition by rectifying with polytetrafluoroethane when chemical analysis shows that the alkalinity of the bath is excessive. The polytetrafluoroethane is added to the molten bath by mechanically submerging small portions at a time in the bath. Sufficient polytetrafluoroethane is added to neutralize the bath and the process is repeated as often as necessary to keep the bath neutral. When the salt bath is kept neutralized as described, an article of steel having the above composition and having a surface free from pits and decarburization will when heated for an hour at 1500° F. show no material change in the surface quality.

*Example III*

A salt bath composed of anhydrous barium chloride is used to harden a tool steel containing 0.73% carbon; 0.30% manganese, 4.51% chromium, 18.21% tungsten, 0.75% molybdenum, 0.26% silicon, 1.25% vanadium by heating at a temperature of 2350° F. The barium chloride is kept in a neutral condition with respect to the tool steel by rectifying the molten bath with sodium fluosilicate when the alkalinity becomes excessive, about 3% calculated as barium oxide. The sodium fluosilicate is added in small portions until tests indicate that the alkalinity is neutralized. After heating the tool steel for an hour at 2350° F. in the barium chloride kept neutral as described, the surface will be found to be substantially the same as the original from the standpoint of decarburization and surface defects.

*Example IV*

A salt bath composition for the heat treatment of steel is kept constantly neutral and nondecarburizing to the steel by the inclusion of sodium fluoborate in the following mixture, viz. barium chloride 55 parts; potassium chloride 25 parts; sodium chloride 20 parts and sodium fluoborate  $\frac{1}{16}$  part—all parts taken by weight.

*Example V*

A salt bath composition for the heat treatment of copper is kept constantly neutral to the copper and avoids pitting and etching by the inclusion of sodium fluoborate in the following mixture, viz. barium chloride 55 parts, potassium chloride 25 parts, sodium chloride 20 parts and sodium fluoborate  $\frac{1}{16}$  part—all parts taken by weight.

What I claim is:

1. A new composition of matter for the heat treatment of steels, copper alloys and nickel alloys, consisting of barium chloride 55 parts; potassium chloride 25 parts; sodium chloride 20 parts and sodium fluoborate  $\frac{1}{16}$  part, all taken by weight.

2. A composition of matter for the heat treatment of metal consisting of a mixture of halide salts together with a compound added in a proportion of at least  $\frac{1}{16}$  part compound to 100 parts halide salts, said compound being non-gaseous at standard temperature and pressure and consisting of three elements, one of which is fluorine, another which is taken from the alkali and alkaline earth metal group and a third element chosen from a group consisting of boron, carbon, and silicon.
3. A composition of matter for the heat treatment of steel in a bath consisting of a mixture of halide salts with at least  $\frac{1}{16}$  part an alkali metal fluoborate salt, non-gaseous at standard temperature and pressure, to 100 parts halide salts.
4. A composition of matter for the heat treatment of steel in a bath consisting of a mixture of halide salts with at least  $\frac{1}{16}$  part an alkali-earth metal fluoborate salt, non-gaseous at standard temperature and pressure, to 100 parts halide salts.
5. A composition of matter for the heat treatment of steel in a bath consisting of a mixture of alkali and alkaline earth halides with at least  $\frac{1}{16}$  part an alkali metal fluoborate salt, non-gaseous at standard temperature and pressure, to 100 parts alkali and alkaline earth halides.
6. A composition of matter for the heat treatment of steel in a bath consisting of a mixture of alkali and alkaline earth halides with at least  $\frac{1}{16}$  part an alkali earth metal fluoborate salt, non-gaseous at standard temperature and pressure, to 100 parts alkali and alkaline earth halides.
7. A composition of matter for the heat treatment of steel in a bath consisting of a mixture of alkali halides together with at least  $\frac{1}{16}$  part an alkali metal fluoborate salt, non-gaseous at standard temperature and pressure, to 100 parts alkali halides.
8. A composition of matter for the heat treatment of steel in a bath consisting of a mixture of alkali halides with at least  $\frac{1}{16}$  part an alkali-earth metal fluoborate salt, non-gaseous at standard temperature and pressure, to 100 parts alkali halides.
9. A composition of matter for the heat treatment of steel in a bath consisting of a mixture of alkaline earth halides with at least  $\frac{1}{16}$  part of an alkali metal fluoborate salt, non-gaseous at standard temperature and pressure, to 100 parts alkaline earth halides.
10. A composition of matter for the heat treatment of steel in a bath consisting of a mixture of alkaline earth halides with at least  $\frac{1}{16}$  part of an alkali-earth metal fluoborate salt, non-gaseous at standard temperature and pressure, to 100 parts alkaline earth halides.
11. A composition of matter for the heat treatment of steel in a bath consisting of a mixture of halide salts with at least  $\frac{1}{16}$  part an alkali metal fluosilicate, non-gaseous at standard temperature and pressure, to 100 parts halide salts.

ISAAC LAIRD NEWELL

**REFERENCES CITED**

The following references are of record in the file of this patent:

| UNITED STATES PATENTS |               |               |
|-----------------------|---------------|---------------|
| Number                | Name          | Date          |
| 2,394,777             | Holden et al. | Feb. 12, 1946 |
| 2,400,511             | Holden        | May 21, 1946  |